

# UNITED STATES PATENT OFFICE

RUSSELL HANDY, OF MANVILLE, RHODE ISLAND, ASSIGNOR OF ONE-HALF  
TO GEORGE DRAPER & SONS, OF HOPEDALE, MASSACHUSETTS.

## ART OF MANUFACTURING COTTON YARN.

SPECIFICATION forming part of Letters Patent No. 245,294, dated August 9, 1881.

Application filed June 9, 1881. (No model.)

*To all whom it may concern:*

Be it known that I, RUSSELL HANDY, of Manville, county of Providence, and State of Rhode Island, have invented an Improvement in the 5 Art of Manufacturing Cotton Yarn; and I do hereby declare that the following specification is a full, clear, and exact description thereof.

This invention has for its object an improved method of manufacturing cotton yarn, where- 10 by its strength is materially increased and its cost of production decreased.

In ordinary practice, the sliver from the rail- 15 way-head or drawing-frames is taken to a roving-frame, when it is reduced in size by draw- ing, and is twisted only sufficiently to prevent it stretching as it is unwound from the bobbin. The roving so made by one frame is put through one or more similar operations to the one just 20 described until the roving is of proper size to be taken to the spinning frame or mule, the draft of which has been so limited as not to exceed twelve to one, or, in other words, the draft of which has not been greater than to draw the roving out twelve times its length. Not more 25 than eight to one has been the commonly-established draft, and it has been considered by the best authorities in manufacturing that draft in excess of such amount was injurious in the production of good uniform yarn, and this is an 30 incontrovertible fact where a single roving is applied to the spinning frame or mule. Two rovings have heretofore been combined to be manufactured into yarns; but in all such cases the size of the rovings respectively has been 35 reduced before subjecting them to the spinning frame or mule by prior operations, so that the aggregated two rovings were equal only in size to a single roving, suitable for making, with the established regulation draft, the re- 40 quired number of yarn, and in manufacturing such combined rovings into yarn the draft has not been increased over what would be em- ployed in manufacturing into the same num- 45 ber of yarn a single roving of double the size. Every additional operation for the reduction of the size of roving not only involves the em- ployment of expensive machinery, but weak- 50 ens the product from the effect of the strain to which the fibers of the cotton are subjected in being drawn upon or past each other in the roving-machinery.

I have discovered that by combining two rovings, each of which is, say, No. 3½, or the size that would be proper to employ to make its standard number of, say, No. 28 yarn with a draft of, say, 55 eight to one, I can, doubling the draft—say, sixteen to one—produce the same number of yarn that would be obtained from either of the single rovings by the regulation draft, and that such yarn will be of greatly-increased 60 strength and improved quality as to even- ness. By this method I greatly economize the manufacture of yarns by dispensing with all the intermediate mechanical operations which have been heretofore invariably employed and 65 deemed essential for the proportionate reduction of the size of the roving when yarns from two combined rovings have been made. More- over, I have found that the same general law is applicable to the manufacture of yarn of 70 any given number, by combining two rovings of any number and proportionably increasing the draft over the regulation draft for such single roving, so as to produce the required number of yarns—as, for example, if I take two 75 coarser rovings of No. 2, I can produce a No. 28 yarn by giving to such combined rovings a draft of, say, twenty-eight to one. I have by my process practically drawn two combined rovings on the spinning-frame with a draft of 80 from eighteen to twenty to one, and I have also spun yarn with success from two rovings with a draft as high as twenty-six to one, and I am convinced that by combining three rovings the draft can be proportionably increased 85 with excellent results.

In the manufacture of fine yarns, where double roving has heretofore been used of high numbers, I propose to use coarse roving, and thus dispense with many expensive machines 90 and the labor required to attend the same and the cost of power to drive them, and at the same time obtain a better product as the result of diminishing the number of deteriorat- 95 ing mechanical operations. I have taken the same roving, suitable for both fine and coarse yarns, and drawn it singly with ordinary draft, and drawn it doubled with double draft, and, as a result, all numbers or sizes of roving treated by my process last referred to have been made 100 so much more even that the variation in the size of one thread compared with others has

been reduced one-half over the ordinary variation, and the strength of the yarn has been increased from ten to twenty-five per cent. I have practiced this in several mills with this 5 invariable result.

I prefer, for the greatest economy in the production of rovings, to produce them on the slubbing-frame by the process described in my patent of the United States, No. 166,001, dated o July 27, 1875, to which reference may be had; but the rovings may be produced by the process common before my said patent drawing-frames being employed; but in this, my present invention, as in that, ordinary drawing-5 frames may be dispensed with.

I claim—

The improvement in the art of manufacturing any prescribed number or size of cotton

yarn or thread, which consists in combining or drawing together two or more rovings, each 20 of which is of the size proper to be used for producing, when worked alone, such prescribed number of yarn, and subjecting such combined rovings during spinning to a draft in excess of the draft proper to be given for like sizes of 25 rovings when worked singly, and sufficient to draw out the combined rovings to produce under the spinning operation such prescribed number of yarn, substantially as described.

In testimony whereof I have signed my name 30 to this specification in the presence of two subscribing witnesses.

RUSSELL HANDY.

Witnesses:

THOMAS ROBINSON,  
JAMES S. UTLEY.